

Patented Oct. 21, 1952

2,614,927

# UNITED STATES PATENT OFFICE

2,614,927

## RAPID PROCESSING OF PHOTOGRAPHIC MATERIALS

Geoffrey Broughton and Robert N. Woodward,  
Rochester, N. Y., assignors to Eastman Kodak  
Company, Rochester, N. Y., a corporation of  
New Jersey

No Drawing. Application June 1, 1949,  
Serial No. 96,627

7 Claims. (Cl. 95—6)

1

This invention relates to photography and particularly to the rapid processing of photographic materials.

Photographic processing of the customary silver halide emulsions after exposure, includes the essential steps of development, fixing, washing and drying. Optional steps such as reduction, toning, etc., may be included but are not essential to the formation of a photographic image. These essential steps consume an appreciable amount of time, and in many cases the time required for completion of each step cannot be shortened without lessening the quality of the final picture. For example, it is well known that incomplete washing of silver images to remove hypo causes the images to eventually fade on aging.

A rapid processing method capable of producing stable photographic prints of high quality would be a desirable improvement over the customary processing methods. It is therefore the principal object of the present invention to provide a rapid method for processing silver halide emulsions. Other objects will appear from the following description of our invention.

These objects are accomplished by the technique described below, an essential feature of which is the treatment of the developed image with a stabilizing agent which avoids the necessity of washing.

According to our invention, a silver halide emulsion, preferably a gelatino-silver halide emulsion, containing a developing agent is exposed in the usual manner and is then developed by treatment with an alkaline solution. If the emulsion is coated on a paper or other porous support, it is desirable to wipe the surface of the emulsion with a sponge, a rubber roll, or other applicator wet with the alkaline solution so that the paper support is not soaked with developing solution. Another method of applying the solution includes pressing the exposed layer against a pad moistened with the alkaline solution, as will be described hereinafter.

Stabilizing agents which we may employ are compounds containing double-bonded sulfur or an SH linkage; for example, alkali metal and ammonium thiocyanates, thioureas and thioglycollic acid as well as alkali metal and ammonium thiosulfates. These agents are generally used in lower concentration than they would be in normal fixing procedure where the emulsion is washed after fixing.

Specific stabilizing agents which we may use, together with the useful concentrations in aqueous solution are as follows:

Per cent

Potassium thiocyanate 10  
Ammonium thiocyanate 5  
Sodium thiosulfate 10

2

Per cent

Potassium thiosulfate 10  
Ammonium thiosulfate 10  
Thiourea 2  
Ethylene thiourea 2  
Propylene thiourea 2  
Thioglycollic acid (Na salt) 10

These concentrations are based on a treatment or immersion time of about 30 seconds. Lower concentrations might be used with longer application or immersion times. The upper limit of concentration is defined by the solubility of the reagent and the general tendency towards crystallization in the photographic material when very high concentrations are used.

The time of treatment will vary with the nature of the film (that is, the grain size and chemical composition), the temperature of treatment and the manner of application of the stabilizing solution. The time necessary for the application of a given stabilizing solution may be readily judged by inspection of the emulsion layer. It is necessary that the silver halide shall have disappeared from the emulsion and the disappearance of the halide, which indicates the formation of a stable complex with the stabilizing compound, may be determined by inspection of the emulsion layer. When the silver halide has just disappeared from the emulsion, stabilization is complete.

The thiosulfates and thioureas are used in acid solution, the thioglycollic acid in alkaline solution, and the thiocyanates in either acid or alkaline solution. The following examples are illustrative:

### Example 1

An emulsion suitable for use in our invention is made as follows: Solutions are made of (A) 25 grams of gelatin in 1 liter water at 40° C. (B) 100 grams silver nitrate in 500 cc. water at 20° C. and (C) 35 grams of sodium chloride in 500 cc. of water. Solutions B and C are simultaneously run into solution A at a uniform rate while stirring the latter over a period of about 10 minutes; solution B preferably not being allowed to run in faster than C. Thereafter, 150 grams of gelatin in 1500 cc. of water at 40° C. are added. 25 grams of 3,4-dihydroxy diphenyl are then dissolved in 250 cc. of methyl alcohol. This solution is slowly added to the above emulsion with stirring and as a result the developing agent becomes dispersed in the emulsion in minute crystals. Preparatory to coating an emulsion layer, formaldehyde or other gelatin hardening agent may be added to the emulsion and the emulsion is coated on a paper support over an area of about 500 square feet. The dried product is then exposed in any of a number of ways to a subject; for example, to a negative by contact

or projection or if the subject is printed matter on a paper base, the exposure may be made by means of reflex printing methods or in any other manner desired. Thereafter the exposed element containing developing agent in the emulsion layer is treated for about 30-60 seconds with an aqueous alkaline solution; for example, of the following composition:

|                                  | Grams |
|----------------------------------|-------|
| Sodium carbonate                 | 50    |
| Sodium hydroxide                 | 5     |
| Sodium thiosulfate (crystalline) | 2     |
| Potassium bromide                | 8-16  |
| Water to 1 liter.                |       |

Both the thiosulfate and bromide in the above formula tend to prevent fog on development of the exposed element. While the alkaline solution can be applied with a sponge, a preferred method includes pressing the exposed layer against the surface of a pad of cloth, paper, felt, sponge rubber, or a water-permeable hydrophilic colloid layer such as gelatin, gum arabic or polyvinyl alcohol moistened with the alkaline solution. A polyvinyl alcohol pad can be prepared by coating a paper support with an aqueous solution of polyvinyl alcohol containing a melamine-formaldehyde condensation product as a hardening agent. A typical coating composition is the following:

|                                |       |      |
|--------------------------------|-------|------|
| Polyvinyl alcohol              | grams | 237  |
| Water                          | cc    | 2300 |
| Melamine-formaldehyde solution | cc    | 135  |
| pH                             |       | 4    |

The melamine-formaldehyde solution in the above formula is prepared by reacting 25 cc. of 20 per cent formaldehyde at pH of 7 with six grams melamine and 100 cc. of water at 80° C., cooling to 40° C., adding 100 cc. of water and adjusting the pH to 7. After the hardening solution has been added to the aqueous polyvinyl alcohol solution, the pH is adjusted to 4 to improve hardening.

The exposed and developed but unfixed element is then treated for about 30-60 seconds with a solution of a stabilizing agent for our invention of which the following is typical:

|                    | Grams |
|--------------------|-------|
| Sodium sulfite     | 15    |
| Sodium bisulfite   | 45    |
| Sodium thiosulfate | 150   |
| Water to 1 liter.  |       |

As in the above development step, this stabilization treatment may be accomplished by swabbing or preferably rolling the developed element down onto a pad moistened with the stabilizing solution. Since the stabilization step converts all residual silver halide to the inactive state, the element need now be only dried without further treatment to provide a stable print.

#### Example 2

Another faster emulsion suitable for use in our invention is made from the following solutions: (A) 25 grams gelatin in 1 liter water at 40° C.; (B) 100 grams silver nitrate dissolved in 500 cc. water at 20° C.; (C) 72 grams potassium bromide in 500 cc. water at 20° C. Solutions B and C are simultaneously run into solution A with stirring and afterwards a solution of 200 grams gelatin in 2 liters water at 40° C. is added. A suitable surface-active agent may then be added and the pH adjusted to 5.0. Thereafter, a solution of 25 grams of 3,4-dihydroxy-diphenyl in 250 cc. of methyl alcohol is added with stirring. Prepara-

tory to coating the emulsion, formaldehyde may be added as a hardener and the emulsion is coated on a paper support over an area of about 300 square feet. The product is then exposed, developed and stabilized as described in Example 1 and the prints dried without washing. The resulting image was stable and no discolorations of the emulsion layer appeared when the prints were incubated or exposed to ultra-violet light for moderate periods of time.

The advantages of our process will now be apparent. One of the chief advantages lies in the fact that the usual developing solution containing developing agent is dispensed with. As is well known, the usual developing solutions have a very short life partly because the developing agent therein readily oxidized in the presence of air even when restrainers are incorporated in the developer. Therefore, the worker must continually change developing solutions. Since we incorporate the developing agent into the emulsion layer, there is no need to use a developing agent in the alkaline treating solution although this can be done if desired. Also, with the elimination of the usual washing step, the total processing time for a print has been decreased from an hour or more to a matter of two to three minutes, yet the images obtained are relatively stable and show little discoloration on exposure to ultraviolet light or aging under adverse conditions; for example, as long as nine days at 120° F. and 98 per cent relative humidity. Also the prints thus stabilized are more permanent than similar prints which have been processed by normal techniques and partially washed.

The developing agents may be incorporated into emulsions of types other than shown in the above examples; for example, the well-known direct positive type of emulsion, particularly those disclosed in the Kendall et al. U. S. Patent application Ser. No. 35,987, filed June 29, 1948, now Patent No. 2,541,472, issued February 13, 1951, may contain the developing agent in the amounts indicated herein and be processed in a manner similar to that described in the above examples. The result, of course, is to obtain a direct positive stabilized image from the original copy and the print has the stability indicated above.

The concentration of developing agent in the above emulsions is dependent in part on the result desired but can be of the order of 350 grams per kg. of silver nitrate, converted to silver halide, used in making the emulsion, to obtain good density or about 250 grams per kg. of silver nitrate to obtain adequate density and an emulsion having optimum keeping properties.

As mentioned, our emulsions are preferably gelatino-silver halide emulsions. However, we are not limited thereto since other water-permeable organic colloid vehicles may be used for dispersing the silver salt and developing agent, e. g., polyvinyl alcohol, partially hydrolyzed polyvinyl esters and cellulose esters, etc.

The developing agents useful in emulsions processed according to our invention include, for example, 3,4-dihydroxy diphenyl; 2,5-dihydroxy diphenyl; 2,3-dihydroxydiphenyl and 5,6,7,8-tetrahydronaphthohydroquinone. These developing agents are substantially insoluble in water and are representative of a group of fairly insoluble developing agents soluble to the extent of .005 to 1.0 gram per hundred cc. of a phosphate-citric acid buffer solution of pH 5.0 prepared from a 1.5 per cent solution of sodium dihydrogen phosphate and sufficient citric acid

to bring the pH to 5.0. The three first-mentioned developing agents have solubilities within the range of from about .01 to 0.1 gram per hundred cc. of the buffer solution and are thus preferred. The developing agents are classified as above in terms of their solubility in a buffer solution because this approximates the solubility behavior of the preferred compounds, particularly when used in emulsion layers in our process. Other more soluble developing agents, for example, hydroquinone, pyrocatechol, and p-methylaminophenol sulfate, may be used in the emulsion layer but are less preferred partly because of their diffusion characteristics in emulsion layers which allow them to transfer to pads used in the processing operations and further because they more readily oxidize and tend to stain the print.

The stabilizing agents mentioned may be used as in the above examples in aqueous solution but it is preferable to make the stabilization bath acid to counteract alkali present in the developing solution. The alkali of the developing solution is not especially critical since carbonate, caustic alkali and borates all give useful results, although, as is apparent, strong alkali is preferred in the alkaline treating solution since it will increase the speed of development of emulsion layers containing weak developing agents such as the dihydroxy diphenyl compounds.

A precaution to be taken particularly if the pad method of processing is used, is to use well-hardened emulsions to prevent the emulsion from adhering to the surface of the pad. In case the emulsion has not been hardened sufficiently prior to processing, this can be done with a formaldehyde hardening bath before or after the development step or in any other suitable way.

Although the emulsion may be immersed in the alkaline and stabilizing solutions, we prefer merely to moisten the surface of the exposed emulsion with these solutions except in the case of films and plates. Thus in the case of paper supports, the support does not become wet and the drying time is greatly reduced.

It will be apparent from the foregoing description of our invention that a substantial proportion of the silver compounds remains in the emulsion after the stabilizing treatment. This differs from the customary fixing and washing in which the intent is to remove the residual silver halide from the emulsion.

It will be understood that the examples and modifications described herein are illustrative only and that our invention is to be taken as limited only by the scope of the appended claims.

We claim:

1. A rapid process for the formation of an image in a photographic emulsion layer which comprises exposing a silver halide emulsion layer containing a developing agent selected from the group consisting of 3,4-dihydroxy diphenyl; 2,5-dihydroxy diphenyl; and 2,3-dihydroxy diphenyl, developing a silver image in said exposed layer by treatment with an alkaline solution, and immediately thereafter stabilizing said layer with a solution of a compound selected from the group consisting of alkali metal and ammonium thiocyanates and thiosulfates, thioureas and thioglycolic acid, and drying said layer without further treatment.

2. A rapid process for the formation of an image in a photographic emulsion layer which comprises exposing a silver halide emulsion

layer containing a silver halide developing agent selected from the group consisting of 3,4-dihydroxy diphenyl; 2,5-dihydroxy diphenyl; and 2,3-dihydroxy diphenyl, developing a silver image in said exposed layer by treatment with an alkaline solution, and immediately thereafter stabilizing said layer with a solution of an alkali metal thiosulfate, and drying said layer without further treatment.

10 3. A rapid process for the formation of an image in a photographic emulsion layer which comprises exposing a silver halide emulsion layer containing a silver halide developing agent selected from the group consisting of 3,4-dihydroxy diphenyl; 2,5-dihydroxy diphenyl; and 2,3-dihydroxy diphenyl, developing a silver image in said exposed layer by treatment with an alkaline solution, and immediately thereafter stabilizing said layer with a solution of an alkali

15 metal thiocyanate, and drying said layer without further treatment.

15 4. A rapid process for the formation of an image in a photographic emulsion layer which comprises exposing a silver halide emulsion layer containing a silver halide developing agent selected from the group consisting of 3,4-dihydroxy diphenyl; 2,5-dihydroxy diphenyl; and 2,3-dihydroxy diphenyl, developing a silver image in said exposed layer by treatment with an alkaline solution, and immediately thereafter stabilizing said layer with a solution of an alkali

20 metal thiocyanate, and drying said layer without further treatment.

25 4. A rapid process for the formation of an image in a photographic emulsion layer which comprises exposing a silver halide emulsion layer containing a silver halide developing agent selected from the group consisting of 3,4-dihydroxy diphenyl; 2,5-dihydroxy diphenyl; and 2,3-dihydroxy diphenyl, developing a silver image in said exposed layer by treatment with an alkaline solution, and immediately thereafter stabilizing said layer with a solution of a thiourea, and drying said layer without further treatment.

30 5. The process of claim 1 wherein the silver halide emulsion is a direct-positive emulsion.

35 6. The process of claim 2 wherein the emulsion is a direct-positive emulsion.

7. A light sensitive photographic element comprising a support having thereon a direct-positive silver halide emulsion layer containing a substantially water-insoluble silver halide developing agent selected from the group consisting of 3,4-dihydroxy diphenyl; 2,5-dihydroxy diphenyl; and 2,3-dihydroxy diphenyl.

45 45 GEOFFREY BROUGHTON.  
ROBERT N. WOODWARD.

#### REFERENCES CITED

The following references are of record in the 50 file of this patent:

#### UNITED STATES PATENTS

| Number    | Name            | Date           |
|-----------|-----------------|----------------|
| 742,405   | Eichengrun      | Oct. 27, 1903  |
| 1,582,050 | Johnson         | Apr. 27, 1926  |
| 2,005,837 | Arens           | June 25, 1935  |
| 2,090,484 | Ostromeslinsky  | Aug. 17, 1937  |
| 2,126,516 | Szasz           | Aug. 9, 1938   |
| 2,214,446 | Albers          | Sept. 10, 1940 |
| 2,397,924 | Crabtree et al. | Apr. 9, 1946   |
| 2,409,107 | Crabtree et al. | Oct. 8, 1946   |
| 2,412,674 | Crabtree et al. | Dec. 17, 1946  |
| 2,448,857 | Brice           | Sept. 7, 1948  |
| 2,453,346 | Russell         | Nov. 9, 1948   |
| 2,541,472 | Kendall et al.  | Feb. 13, 1951  |

#### FOREIGN PATENTS

| Number  | Country       | Date          |
|---------|---------------|---------------|
| 549,956 | Great Britain | Dec. 16, 1942 |

#### OTHER REFERENCES

Abstract File No. 594,589, Yackel, filed May 18, 1945, published July 26, 1949 in Official Gazette, Patent Office.